

# UNITED STATES PATENT OFFICE.

LEON LILIENFELD, OF VIENNA, AUSTRIA-HUNGARY, ASSIGNOR TO GEORGE HAROLD WINTERBOTTOM, OF HORTON HOUSE, NEAR NORTHAMPTON, ENGLAND.

## PROCESS FOR PRODUCING IMPRESSIONS FAST TO WATER ON TEXTILE FABRICS.

No. 888,516.

Specification of Letters Patent.

Patented May 26, 1908.

Application filed January 8, 1908. Serial No. 409,844.

*To all whom it may concern:*

Be it known that I, LEON LILIENFELD, chemist, a subject of the Emperor of Austria-Hungary, and a resident of Vienna, in the 5 Empire of Austria-Hungary, VIII, Zeltgasse 1, have invented a Process for Producing Impressions Fast to Water on Textile Fabrics; and I do hereby declare the following to be a full, clear, and exact description of the invention, such as will enable others skilled in the 10 art to which it appertains to make and use the same.

The processes heretofore known for producing impressions fast to water on textile fabrics by use of solutions of cellulose nitrates (nitrocelluloses) or celluloid, or cellulose acetates, (acetyl-celluloses) in solvents of comparatively low boiling-point such as amyl-acetate or formate, have been difficult to 15 bring into general use, because the layers of nitrocellulose or acetyl-cellulose produced on the textiles in the ordinary manner, when of the required thickness, deprive the textile fabrics of their softness to the touch and 20 make them feel more or less stiff, hard or like paper.

Even the addition of various softening agents has not given an entirely satisfactory result because the harshness to the touch has 25 not been sufficiently improved thereby; moreover, the effect of such agents is deleterious to the fastness of the materials to friction or to the brilliancy of the product, or to their fastness to water or to all these qualities.

According to the present invention the combinations of nitrocellulose or celluloid or cellulose acetates with organic acid esters of high boiling-point, more particularly the 30 esters of phthalic acid, are especially suitable for imparting resistance to water to impressions on textile fabrics, particularly to the

effects known as "silk finish." Textile fabrics dressed or coated with such combinations do not lose their softness to the touch when 45 sufficient quantities of the combinations are applied. These latter have an extremely high capacity of imparting resistance to water to textile materials when these have been provided with designs applied by means 50 of silk-finishing on goffering rolls.

To the coating compositions there may be also added known dressing or fixing agents such as for example, glue, (gelatin), resins or albuminous substances, according to the nature of the solvents. For example, 100 parts of nitro-cellulose or celluloid are dissolved together with 50 to 150 parts of ethyl phthalate, in a suitable solvent, such as methyl alcohol, acetone, ethyl alcohol alone or mixed 55 with acetic anhydrid, ethyl acetate or another ester of low boiling-point such as amyl-acetate or butyl acetate, the solution is applied as a dressing composition to the textile fabric before or after the goffering process. 60

What I claim as my invention and desire to secure by Letters Patent is:

The herein described process for producing impressions fast to water on textile fabrics by treating the fabric, before or after the goffering process, with combinations of nitrocellulose or acetyl-cellulose, either alone or mixed together or with other dressing materials, with organic acid esters of high boiling-point, particularly with a phthalic acid ester, 75 substantially as described.

In testimony whereof I have signed my name to this specification in the presence of two subscribing witnesses.

LEON LILIENFELD.

Witnesses:

WENZEL SINKE,  
ROBERT S. HEINGARTNER.